

## UNITED STATES PATENT OFFICE

JOSEPH NÜSSLIN, OF LUDWIGSHAFEN-ON-THE-RHINE, GERMANY, ASSIGNOR, BY  
MESNE ASSIGNMENTS, TO GENERAL ANILINE WORKS, INC., OF NEW YORK, N. Y., A  
CORPORATION OF DELAWARE

## DYEING FIBROUS MATERIALS

No Drawing. Application filed October 16, 1925, Serial No. 62,932, and in Germany October 30, 1924.

I have found that the treatment of fibrous materials with dyeing liquors is considerably improved if the dyeing liquors are prepared with an addition of a small quantity of sulfonic acids of such aromatic hydrocarbons as contain alkyl groups with more than two carbon atoms, especially of naphthalene and similar hydrocarbons with several benzene rings containing propyl or butyl (normal or iso) groups.

The term fibrous materials is employed in a broad way including all textile fibres, for example wool, cotton, natural and artificial silk and the like, also jute, straw, paper, leather, hides, furs, feathers and the like, and the dyeing process is the usual one which is carried out in a dyeing liquor as contrasted with the little usual dyeing in the lather.

The said sulfonic acids enable the fibrous materials to be wetted very rapidly in an excellent manner and make it unnecessary to apply any special boiling operation to the goods before introducing them into the dye-bath. The said sulfonic acids have the advantage of being insensitive to acids or hard water. Consequently they can be employed not only in alkaline or neutral dyebaths but also in acid baths. In any case very uniform dyeings are produced even with dyestuffs which make this very difficult when dyed in the usual way.

The sulfonic acids may be employed as such or in the state of their salts. Sometimes it may be advantageous to use the free sulfonic acids or their salts in mixture with aliphatic alcohols, especially the higher members of this group that is to say such as contain more than 3 carbon atoms.

The following examples will more fully explain the manner of carrying the invention into practice which, however, I do not wish to limit in any way to these examples. The numbers after the trade names of the dyestuffs employed correspond to those of the Color Index, 1st edition, 1924.

## Example 1

A piece of woollen cloth is introduced into a lukewarm dyebath prepared from 0.6 per cent of Cyananthrol BGA (1077), 0.6 per

cent of Azoflavine FF (147), 0.2 per cent of Sorbina Red (54), 10 per cent of Glauber's salt, 2 to 3 per cent of sulfuric acid of 66 degrees Baumé and 2 per cent of isopropylated naphthalene sulfonic acid, sodium salt, and stirred for about 10 minutes. The bath is then heated to the boil in the course of  $\frac{1}{4}$  to  $\frac{1}{2}$  hour and after being kept boiling for one hour it is allowed to cool. The goods are then well rinsed.

Or the goods, for example hats in a half planked state, carbonized or impure, are wetted in the evening before dyeing by handling for half an hour at 70 degrees centigrade in a bath containing 0.5 per cent of isopropylated naphthalene sulfonic acid, sodium salt, left in the bath during the night and dyed in the next morning in the above described manner with an addition of 0.5 per cent of the said sulfonic acid sodium salt, 20 per cent of Glauber's salt and the necessary quantity of acid to the dyebath.

If instead of the sodium salt the free sulfonic acid is employed, the sulfuric acid may be left out wholly or partly.

## Example 2

Unboiled, raw cotton yarn is directly introduced at 50 degrees to 60 degrees centigrade into a dyebath containing 10 per cent of Indanthrene Blue RS (1106) and, in each litre, 12 cubic centimetres of caustic soda lye of 40 degrees Baumé, 1.5 grams of dry sodium hydrosulfite and 2 to 4 grams of isopropylated naphthalene sulfonic acid, sodium salt, dyed for  $\frac{3}{4}$  to 1 hour as usual with indanthrene dyestuffs and finished by rinsing and soaping in a boiling bath.

## Example 3

Unboiled, raw cotton yarn is directly introduced into a boiling dyebath prepared from 3 per cent of Oxamine Blue B (515) and, in each litre, 10 grams of Glauber's salt and 1 to 3 grams of isopropylated naphthalene sulfonic acid, sodium salt. The goods are dyed for 1 hour in the manner usual for direct dyestuffs and finished as usual.

The developing of dyestuffs on the fibrous materials may be effected in a similar manner.

Instead of the sodium salt of isopropylated naphthalene sulfonic acid, other soluble salts or the free acids or butylated naphthalene sulfonic acid or their salts may be employed.

I claim:

1. A composition of matter suitable for dyeing fibrous materials, comprising an aliphatic alcohol and a naphthalene sulfonic acid containing at least one alkyl group with more than two carbon atoms.
2. A composition of matter suitable for dyeing fibrous materials, comprising an aliphatic alcohol with more than three carbon atoms and a naphthalene sulfonic acid containing at least one alkyl group with more than two carbon atoms.
3. Baths, suitable for dyeing which are characterized in addition to the content of a coloring matter by an addition of a sulfonic acid of an aromatic hydrocarbon containing in the nucleus at least one alkyl group with more than 2 carbon atoms and of an aliphatic alcohol.
4. Baths, suitable for dyeing which are characterized in addition to the content of a coloring matter by an addition of a naphthalene sulfonic acid containing in the nucleus at least one alkyl group with more than 2 carbon atoms, and of an aliphatic alcohol with more than three carbon atoms.
5. A composition of matter suitable for dyeing fibrous materials comprising an aliphatic alcohol and a naphthalene sulfonic acid containing at least one isopropyl group.
6. A composition of matter suitable for dyeing fibrous materials comprising an aliphatic alcohol with more than three carbon atoms and a naphthalene sulfonic acid containing at least one isopropyl group.
7. A composition of matter suitable for dyeing fibrous materials comprising an aliphatic alcohol and a naphthalene sulfonic acid containing at least one butyl group.
8. A composition of matter suitable for dyeing fibrous materials comprising an aliphatic alcohol with more than three carbon atoms and a naphthalene sulfonic acid containing at least one butyl group.

In testimony whereof I have hereunto set my hand.

JOSEPH NÜSSLEIN.